

April 20, 1926.

1,581,510

C. CAMPBELL

TYPEWRITER RIBBON

Filed Dec. 16, 1924

Fig. 1



Fig. 2



Fig. 3



INVENTOR

CHARLES CAMPBELL

BY

Newell and Spencer.

ATTORNEY

Patented Apr. 20, 1926.

1,581,510

# UNITED STATES PATENT OFFICE.

CHARLES CAMPBELL, OF NEW YORK, N. Y.

## TYPEWRITER RIBBON.

Application filed December 16, 1924. Serial No. 756,363.

*To all whom it may concern:*

Be it known that I, CHARLES CAMPBELL, a citizen of the United States, residing at New York city, N. Y., have invented a certain new and useful Improvement in Type-  
writer Ribbons, of which the following is a clear, full, and exact description.

The present invention relates to type-  
writer ribbons and more particularly to im-  
10 provements in typewriter ribbons made from  
matted or felted plant fibres.

In my Patent No. 1,533,382 of April 14, 1925, I have described a typewriter ribbon made particularly from fibres comprising  
15 mainly the fibres of the Japanese mul-  
berry or *Broussonetia papyrifera*, the in-  
vention being based on the discovery that  
these fibres when felted and incorporated  
20 into the typewriter ribbon material impart  
the necessary tensile strength, enabling the  
ribbon to stand the wear and tear during  
use, and also has the quality of resistance to  
rupture through which it withstands the  
25 pounding of the typewriter keys without  
disintegrating.

As a result of extended experimentation  
with mixtures of fibres I have discovered  
that while fibres other than "*Broussonetia*"  
fibres may be admixed therewith in the  
30 making of typewriter ribbons, the neces-  
sary strength and resistance to pounding,  
being contributed mainly by the "*Brou-  
ssonetia*" fibres, the addition of certain fibres  
in the mixture, such as hemp and jute,  
35 causes a serious interference with the feed-  
ing qualities or ink dispersion through the  
ribbon.

The causes underlying the interference  
with the feeding qualities or "recovery"  
40 properties of the ribbons due to the use of  
certain fibres are not entirely understood.  
I have, however, discovered a means of over-  
coming the difficulties by the admixture of  
a material increasing the feed or flow of ink  
45 through the ribbon after a part is removed  
from the ribbon.

It seems probable that in the use of a type-  
writer ribbon made from textile fabric that  
after a portion of the ink or dope has been  
50 transferred from the ribbon to a paper by  
the impact of the typewriter type on the  
ribbon, the ink from other adjacent parts of  
the ribbon creeps along the fibres thereof  
55 toward the area from which the ink has been  
removed, the flow taking place probably  
through what we would term "capillary

action" which is a variable dependent on  
the amount of space between the fibres, sur-  
face tension and viscosity of the inking  
material, and various other factors. It 60  
seems apparent that the inking material  
flows mainly through the various interstices  
between the fibres and along the surfaces  
thereof, and not through the fibres them-  
selves or by soaking transversely through 65  
the fibres. The amount of inking material  
employed in the ribbon must, of course, be  
limited in order to avoid the filling of the  
type with ink, or producing what is gen-  
erally termed "blotting." It is therefore 70  
apparent that the amount of ink used must  
be between the limits where blotting would  
occur and a certain minimum amount cor-  
responding to what is generally termed  
"ribbon exhaustion," at which point the 75  
amount of ink transferred to the paper is  
insufficient to produce a legible impression,  
and that the larger the amount of ink which  
the ribbon will hold without blotting the  
better the ribbon. 80

Aside from the above considerations, the  
ribbon must, when used, have a rapid rate  
of "recovery"; that is, after removal of ink  
from a particular portion of the ribbon, by  
the striking of the typewriter key, the ink 85  
from the adjacent portions of the ribbon  
must feed to the exhausted or used portion  
thereof at a sufficiently rapid rate so that  
when the same part of the ribbon is again  
struck it will cause an impression on the 90  
paper in the usual way. There must be, in  
other words, a gradual redistribution of the  
ink on the ribbon, after a part thereof is  
removed.

In the making of typewriter ribbons from  
matted or felted plant fibres, particularly  
the *Broussonetia papyrifera*, which imparts  
the desired strength when admixed with  
other fibres, I have found that certain kinds  
of fibres interfere seriously with the feed  
qualities of the ribbon. I have found, for  
example, that fibres having a gummy sur-  
face or "water-shedding" surface interfere  
with the feeding qualities of a ribbon, and  
also decrease the ink holding or absorption  
qualities thereof to a marked degree. Ap-  
parently the capillarity of the space between  
the adjacent fibres is reduced by the inclu-  
sion of fibres having certain water-repellent  
properties, which is inherent in certain 100  
crude, untreated fibres. 110

I have discovered that the above effects

may be wholly avoided, and that the ink capacity of the ribbon may be increased by incorporating in the ribbon a suitable absorption material, as finely comminuted sponge. I have found also that by the use of sponge with plant fibres, particularly the *Broussonetia papyrifera*, or fibres mainly of *Broussonetia papyrifera*, that a remarkable rapidity in "recovery" is attained. Moreover, the increase in capacity or, in other words, the amount of ink which the ribbon is able to hold is greatly increased without attaining the point at which "blotting" commences, or, in other words, the point at which the amount of ink in the ribbon is so great that it will fill the type, thereby producing blots rather than letters. It is apparent, therefore, that by the use of this material which I shall describe more in detail, the life of the ribbon will be greatly increased due to its increased ink capacity, and furthermore, the feeding qualities, or, the rate of "recovery" is greatly increased.

It is the primary object of my invention to provide a ribbon made from plant fibres in which the feeding qualities and rate of "recovery" are greatly increased over that of ribbons of this character heretofore produced.

Another object of the invention is to provide a typewriter ribbon made mainly from fibres of *Broussonetia papyrifera* and containing sponge to improve the working qualities of the ribbon.

With these and other objects in view the invention comprises the various features hereinafter more particularly described and defined in the claims.

The invention is illustrated in the accompanying drawings, in which:

Figure 1 is a view in perspective of a portion of a typewriter ribbon;

Figure 2 is a front view of a typewriter showing a ribbon therein; and

Figure 3 is a diagram indicating the process steps employed for the making of the typewriter ribbon.

In the drawings the numeral 1 indicates a typewriter ribbon and the numeral 2 indicates a typewriter in which the ribbon is used in the ordinary manner.

The fibres of the Japanese mulberry, known as the *Broussonetia papyrifera*, are particularly adapted for the making of typewriter ribbons, by means of which the necessary tensile strength and resistance is attained, and by which the cost of typewriter ribbons is greatly reduced. I found that the ribbons could be made from the fibres composed mainly of the *Broussonetia papyrifera* but having a small proportion of other fibres admixed thereto, without substantial interference with the qualities required in a serviceable ribbon. As above set forth, however, it has been found that cer-

tain fibres, particularly in their crude state, such as jute, interfere, if used in sufficient amounts, with the feeding qualities of the ribbon, even though not added in sufficient amounts to decrease the tensile strength and resistance to pounding to the point where the ribbon would be unsatisfactory as to these properties. If sponge material, which has been very finely comminuted, is added to the fibres of the *Broussonetia papyrifera* or to a mixture of these fibres with other fibres in the beater, it is found that the sponge becomes very thoroughly disseminated among the "Broussonetia" fibres and although it does not add to the tensile strength of the ribbon it increases the feeding qualities thereof. A satisfactory ribbon may be made with a mixture of fibres in which the "Broussonetia" fibre is used in sufficient amount to give the ribbon the required strength, and a sufficient amount of sponge is added to raise the feeding qualities or the "recovering" properties a considerable amount, whereby the addition of jute, and other fibres which would ordinarily reduce the feed or recovery, may be made without detriment.

The proportions which I preferably use in my new ribbon are about 75 per cent of the fibres of the *Broussonetia papyrifera* and 25 per cent of sponge material, although I do not confine myself to these limits. In place of the above proportions I might employ only 10 per cent of the sponge material with 90 per cent of "Broussonetia" fibres. An example of the proportions which may be used with a mixture of fibres in which "Broussonetia" fibres are employed to impart the required tensile strength to the ribbon, is the following: approximately 60 per cent of the "Broussonetia" fibres, 20 per cent of hemp fibre, and 20 per cent of comminuted sponge.

In making up the mix it is preferable to first comminute the sponge material, and then add it to the fibres in the beater. It has been found that the sponge cannot be comminuted sufficiently by the use of the ordinary beater, in which the material is cut by rotating knives. By the use of a beater operating on a somewhat different principle from the ordinary beater, that of hammering the sponge material, it may be comminuted to a point where the various particles of sponge readily interlace, thus acquiring a high degree of adherence to other fibres and even to other shreds or bits of sponge material. After the sponge is sufficiently comminuted it is added to the other fibres in the ordinary beater, and thoroughly mixed, the process being finished in the usual way. By incorporating sponge particles of this character with fibres of *Broussonetia papyrifera* or mixtures thereof with other plant fibres, a very high tensile strength is attained and the feeding proper-

ties of the matted fibre ribbon when inked are greatly enhanced. The sponge material serves also to give increased resiliency to the ribbon, and serves, without doubt, to increase the wearing qualities of the ribbon. These qualities of the ribbon are due in all probability to the peculiar nature of the sponge material which comprises tubes or hollow fibres, which act like springs, giving resiliency to the ribbon, and apparently, because of this property, increasing the "wear" under the type. The sponge material serves also to increase the ink capacity of a ribbon or, in other words, enables the ribbon to soak up a large amount of ink and give it off gradually and quite uniformly during use of the ribbon.

It is to be understood that I have described the preferred method of carrying out my invention but that various changes may be made therein without departing from the spirit or scope of the invention as defined in the claims.

Having thus described the invention what is claimed as new is:

- 25 1. A typewriter ribbon comprising felted plant fibres and ink, and a material to increase the ink feeding or "recovery" properties thereof.
- 30 2. A typewriter ribbon comprising plant fibres and sponge with inking material.
- 35 3. A typewriter ribbon comprising mainly fibres of the *Broussonetia papyrifera* and sponge.
4. A typewriter ribbon comprising more than 50 per cent of plant fibres and comminuted sponge together with inking material.

5. A new article of manufacture adapted for typewriter ribbons which comprises a mixture of comminuted sponge, fibres of *Broussonetia papyrifera* and other plant fibres in which the proportion of "Broussonetia" fibres is at least one-half of the mixture, together with inking material.

6. A process of making typewriter ribbons which comprises pounding or hammering sponge material so as to sufficiently comminute the material to admix with plant fibres, thereafter mixing plant fibres therewith, forming the mixture produced thereby into a thin sheet of proper width and thickness to be adapted for typewriter ribbons, and inking the said sheet.

7. A process of making typewriter ribbons which comprises comminuting sponge by hammering the sponge until the particles thereof are comminuted sufficiently to admix and adhere to plant fibres when added thereto, mixing with the sponge particles thus comminuted plant fibres comprising mainly *Broussonetia papyrifera*, thereafter mixing the fibres and sponge in a beater until a homogeneous mixture is attained, forming thereafter from the mixture a thin sheet suitable for the making of typewriter ribbons and adding inking material.

8. A typewriter ribbon comprising substantially 60 per cent of "Broussonetia" fibres, 20 per cent of hemp fibres, 20 per cent of comminuted sponge, and a suitable amount of inking material.

Signed at New York, N. Y., this 11th day of December, 1924.

CHARLES CAMPBELL.